

# UNITED STATES PATENT OFFICE.

EDWARD D. GLEASON, OF NEW YORK, N. Y., ASSIGNOR, BY MESNE ASSIGNMENTS, TO  
NEU-METALS AND PROCESS COMPANY, OF LONG ISLAND CITY, NEW YORK, A COR-  
PORATION OF NEW YORK.

## IRON, BORON, CARBON, AND COPPER ALLOY,

1,126,629.

Specification of Letters Patent.

Patented Jan. 26, 1915.

No Drawing.

Application filed December 31, 1912. Serial No. 739,454.

To all whom it may concern:

Be it known that I, EDWARD D. GLEASON, of Brooklyn, in the county of Kings, city and State of New York, have invented a  
5 certain new and useful Improvement in Iron, Boron, Carbon, and Copper Alloys, whereof the following is a specification.

It is the object of my invention to provide an alloy that is practically non-corrosive, and which, though hard and tough, 10 may be rolled to sheet form or readily machined without being annealed.

Heretofore it has been assumed, as the result of experience, that copper will not 15 alloy with iron unless the latter be pure. Therefore, as the iron which I employ contains carbon, it is to be understood that the capacity of the copper to alloy therewith is due to the presence of boron.

20 In carrying out my process I prefer to first incorporate the boron in the copper, preferably by subjecting the copper to the action of boron fluorid while the copper is molten, which results in the deposit of boron in the graphitoidal state in the copper when 25 the latter cools. In forming my improved alloy I employ such boron copper in which boron is in excess, viz., in greater quantity than will combine with the copper and as 30 the boron associates with iron as readily as silicon, regardless of the carbon content of the iron, the copper is thereby caused to alloy with the iron and carbon, forming a homogeneous mixture. For instance, by 35 taking 80 parts Bessemer scrap and fusing it in a Hawley-Schwartz furnace and adding 20 parts of copper containing boron in excess, I produce an alloy which may be cast in ordinary sand molds, forming castings 40 which are homogeneous and easily machined. However, it is to be understood that other proportions of low carbon steel, copper and boron may be employed without

departing from the scope of my invention. Therefore, I do not desire to limit myself to the precise proportions or method of procedure herein set forth.

I claim:

1. An alloy containing iron, boron and copper; including approximately 80 per 50 cent. of iron.

2. An alloy containing iron, copper and boron, the principal ingredient of which is iron.

3. An alloy containing iron, boron, and 55 copper; including approximately 80 per cent. of iron, retaining carbon derived from the carbon primarily present in the iron.

4. An alloy containing iron, copper and boron the principal ingredient of which is 60 iron, retaining carbon derived from the carbon primarily present in the iron.

5. An alloy containing iron and copper including boron material in excess of the quantity that will combine with the copper. 65

6. The process of forming an alloy containing iron, copper and boron; which consists in fusing Bessemer scrap with copper containing boron in excess of the quantity that will combine with the copper. 70

7. The step in the process of forming an alloy containing iron, copper and boron which consists in adding to the iron copper including boron in excess of the quantity that will combine with the copper. 75

8. The step in the process of forming an alloy containing iron, copper and boron which consists in adding to the iron copper including boron in the graphitoidal state.

In testimony whereof, I have hereunto 80 signed my name at Philadelphia, Pennsylvania, this thirtieth day of December, 1912.

EDWARD D. GLEASON.

Witnesses:

ANNA ISRAELVITZ,

ETHEL M. IMSCHWEILER.